

# UNITED STATES PATENT OFFICE.

CHARLES P. McCONNELL, OF NEW YORK, N. Y., ASSIGNOR TO WESTERN ELECTRIC COMPANY, OF NEW YORK, N. Y., A CORPORATION OF ILLINOIS.

## LEAD ALLOY.

1,075,661.

Specification of Letters Patent.

Patented Oct. 14, 1913.

No Drawing.

Application filed August 27, 1912. Serial No. 717,274.

*To all whom it may concern:*

Be it known that I, CHARLES P. McCONNELL, a citizen of the United States, residing at 314 West Ninety-ninth street, New York city, in the county of New York, State of New York, have invented a certain new and useful Lead Alloy, of which the following is a full, clear, and exact description.

The subject of my invention is a lead alloy particularly suitable as the material for so-called "tape" used for winding electrical conductors such as telephone switch-board cables, although said alloy may be used for other purposes.

Prior to my invention, tape of the kind above mentioned was usually made entirely of lead rolled to a thickness of substantially .006 of an inch and having a width of substantially .75 of an inch. When made of the alloy hereinafter described, said tape need be only about one-half as thick to obtain the same or greater strength as the tape just mentioned, and its width may be increased by one-third. That is, when my alloy is used, a satisfactory tape need have a thickness of only approximately .003 of an inch, and its width can be 1 inch. It is evident therefore that, compared with the old lead tape, a material saving in lead is effected by the use of my alloy; and it is a fact that this saving is largely in excess of the cost of the metals which are added to form the alloy.

The alloy which forms the subject of my invention is composed of lead, antimony and tin. After careful investigation I have

found that when my alloy is used for the manufacture of tape for winding telephone cables, its preferred composition and the maximum and minimum permissible amounts of the metals forming the alloy are as given in the following table.

|               | Preferred. | Maximum. | Minimum. | 45 |
|---------------|------------|----------|----------|----|
| Lead.....     | 95.00%     | 96.75%   | 93.25%   |    |
| Antimony..... | 4.50%      | 6.00%    | 3.00%    |    |
| Tin.....      | .50%       | .75%     | .25%     |    |
|               | 100.00%    |          |          | 50 |

Having thus described my invention, what I claim and desire to secure by Letters Patent is:

1. An alloy composed of 93.25 to 96.75 per cent. lead, 3 to 6 per cent. antimony, and .25 to .75 of one per cent. tin.
2. An alloy composed of, approximately, 95 per cent. lead, 4.5 per cent. antimony, and .5 of one per cent. tin.
3. As an article of manufacture a thin metallic tape for winding electrical conductors composed of an alloy of approximately 95 per cent. lead, 4.5 per cent. antimony and .5 of one per cent. of tin.

In witness whereof, I hereunto subscribe my name this 26th day of August A. D., 1912.

CHARLES P. McCONNELL.

Witnesses:

ELLA EDLER,  
WALTER F. HOFFMAN.